# EUROPEAN PATENT SPECIFICATION

(11) **EP 0 460 695 B1**
(45) Date of publication and mention of the grant of the patent: **13.11.1996**
(21) Application number: 91109349.0
(22) Date of filing: 07.06.1991
(51) Int. Cl.: C22F 1/00, C22F 1/10, C22C 19/03

(54) **Ti-Ni-C shape memory alloy with a pseudoelasticity and a wide elasticity range**
Pseudoelastische Ti-Ni-C-Formgedächtnislegierung mit einer höheren Elastizitätsgrenze
Alliage pseudo-élastique Ti-Ni-C à mémoire de forme ayant une limite d'élasticité élevée

(30) Priority: 07.06.1990 JP 147325/90
(43) Date of publication of application: 11.12.1991
(73) Proprietor: TOKIN CORPORATION, Sendai-shi Miyagi-ken 982 (JP)
(72) Inventor: Yamauchi, Kiyoshi, Tokin Corporation, Sendai-shi, Miyagi-ken (JP); Sato, Shoichi, Tokin Corporation, Sendai-shi, Miyagi-ken (JP); Takaara, Hideo, Tokin Corporation, Sendai-shi, Miyagi-ken (JP)
(74) Representative: Prüfer, Lutz H., Dipl.-Phys.

(56) References cited:
- EP-A- 0 143 580
- US-A- 4 894 100
- PATENT ABSTRACTS OF JAPAN vol. 12, no. 213 (C-505)(3060) June 17, 1988 & JP-A- 63 11 637 (KEIJIYOU KIOKU GOKIN GIJUTSU KENKYU KUMIAI ) January 19, 1988
- PATENT ABSTRACTS OF JAPAN vol. 14, no. 197 (C-712)(4140) April 23, 1990 & JP-A-2 38 547 (HITACHI METALS LTD ) February 7, 1990
- PATENT ABSTRACTS OF JAPAN vol. 13, no. 255 (C-606)(3603) June 13, 1989 & JP-A-1 56 833 (SUMITOMO ELECTRIC IND LTD ) March 3, 1989
- PATENT ABSTRACTS OF JAPAN vol. 8, no. 279 (C-257)(1716) December 20, 1984 & JP-A- 59 150 047 (HITACHI KINZOKU K.K. ) August 28, 1984
- PATENT ABSTRACTS OF JAPAN vol. 11, no. 222 (C-435)(2669) July 18, 1987 & JP-A- 62 37 353 (HITACHI METALS LTD ) February 18, 1987

## Description

The present invention relates to a method of manufactoring a pseudoelastic spring alloy and, in particular, to improvement of an elasticity range of such an alloy.

It is well known in the art that TiNi alloy and TiNiX alloy, where X is Cu, Cr, etc. indicates a remarkable shape memory effect. This effect is known to be caused by a reverse transition of thermoelastic martensitic transition.

On the other hand, it is also well known that TiNi alloy has a pseudo elasticity which shows flexibility such as rubber. The pseudo elasticity is referred to as an unusual elastic behavior in a paper entitled "CRYSTAL STRUCTURE AND MICROSTRUCTURE OF A COLD WORKED TiNi ALLOY WITH UNUSUAL ELASTIC BEHAVIOR" by Tadaki et al, METALLURGICA, Vol. 14, 1980, Pergamon Press Ltd., pp. 911-914 (Reference 1).

When a stress is loaded or applied to the TiNi alloy wire, the strain of the wire elastically increases by increase of the stress. When the stress exceeds a limit of the elasticity (yield point), the strain of the wire increases at the constant elasticity limit stress. Thereafter, when the stress is removed or unloaded, the strain also decreases with reduction of the internal stress due to discharge of the internal energy stored by the loaded force. Thereafter, the strain is rapidly decreased at a constant internal stress into its elastic condition or state, and then, elastically decreases to recover the original shape.

Accordingly, the TiNi alloy is used in various applications, for example, eye glass frames, catheter guides, orthodontic implements and other spring parts.

However, the TiNi alloy is usually low in the elasticity limit, and therefore, cannot be used for applications requiring a high elasticity limit and the pseudoelasticity.

From JP-A-63-11637 a TiNi alloy is known in which intermediate-phase transformation appears by ageing treatment at ≤ 600°C, 0,5 ∼ 2,0 atomic percent C being substituted for a part of Ni. In a first heat treatment at 800°C a solution treatment is carried out, during a second heat treatment the alloy is heated for 40 hours at 400°C while mechanically restrained onto a copper pipe after the heat treatment. Such an alloy shows improvement in a property of shape memory effect.

From JP-A-2-38547 an alloy constituted of 48,5 to 32,5 atomic percent Ni and the balance Ti is known wherein a part of Ti or Ni is substituted by one ore more kinds of C, O, and N. The alloy is subjected to work hardening and is restricted into a desired shape. In this condition it is subjected to a shape-memory heat treatment.

From JP-A-1-56833 a Ti-Ni shape memory alloy is known having high density and excellent shape memory effects, by packing a powder mixture consisting of Ti, Ni, and additive carbon in a metallic cylindrical body. The cylindrical body is heat treated.

From JP-A-59-150047 a shape memory alloy is known having small hysteresis in the transition of low temperature phase to high temperature phase transformation. Such a property is achieved by adding C, N, or O to shape memory Ti-Ni alloy.

Therefore, it is the object of the present invention to provide a method of manufacturing a pseudo elastic spring alloy having a high elasticity limit and pseudo elastic properties.

This object is achieved by the method as is defined in claim 1. Preferred developments of the method are given in claims 2 to 4.

Preferred embodiments will be explained under reference to the accompanying figures.
Fig. 1 shows stress to strain curves for the maximum 5% tension strain of Ti_{50-x/2}Ni_{50-x/2}Cₓ alloys, where X = 0, 1, 2, 3; and
Fig. 2 shows stress to strain curves for the maximum 5% tension strain of Ti_{49.75-x/2}Ni_{50.25-x/2}Cₓ alloys, where X = 0, 1, 2, 3.

The alloy according to the present invention comprises 0.20-5.0 at% C and the balance Ti and Ni, Ni/Ti = 1-1.08 (50/50-52/48).

The addition of C (carbon) to the TiNi alloy lowers the austenitic and martensitic transition temperatures and also elevates the elasticity limit of the alloy. The minimum amount of C should be 0.2 at%. But, when C is added more than 5.0 at%, the cold working of the alloy is almost impossible. Therefore, the amount of C is limited 5.0 at% or less.

In order to realize the austenitic and martensitic transition points below about 37°C and the pseudoelasticity at about 37°C, the total amount of Ni and C should be 50.0 at% or more. However, the maximum of the total amount is 55.0 at%, preferably 52.0 at%, because the increase of (Ni + C) amount makes the cold working of the alloy difficult.

### Examples

Ingots of alloys containing various amounts of Ti, Ni and C were prepared by the melt method using a high frequency induction furnace.

The ingots were reduced to wires of 1.3mm in diameter by means of hot working and cold working, thereafter solution treated at 950°C for 10 minutes, and reduced to wires of 1.0mm in diameter by means of cold working. The resultant wires were annealed at 500°C for 30 minutes and then subjected to the tensile test at 37°C by means of loading and unloading cycle.

Fig. 1 shows various stress-strain curves of wires of Ti_{50-x/2}Ni_{50-x/2}Cₓ alloys, where x = 0, 1, 2, 3. Fig. 2 also shows various stress-strain curves of wires of Ti_{49.75-x/2}Ni_{50.25-x/2}Cₓ alloys, where x = 0, 1, 2, 3. Referring to Fig. 1, the samples of x = 1, x = 2 and x = 3 according to the present invention have high elasticity limit in comparison with the other sample of x = 0. The elasticity limit is elevated by increase of amount of C. Further, the samples of x = 1, x = 2 and x = 3 have the preferable pseudo elasticity but the sample of x = 0 does not have the pseudo elasticity.

Referring to Fig. 2, it will be understood that samples of alloys Ti_{49.75-x/2}Ni_{50.25-x/2}Cₓ alloys have a tendency similar to samples of Ti_{50-x/2}Ni_{50-x/2}Cₓ.

As mentioned above, the alloy according to the present invention has a pseudo elasticity with a high spring stiffness at a temperature of 37^{o}C so that the alloy can be widely applied as spring materials.

## Claims

1. A method of manufacturing a pseudoelastic spring alloy represented by the chemical formula of Ti_{a-c/2}Ni_{b-c/2}C_{c}, wherein a+b=100, b=50-52, and c=0.20-5.0 in atomic percent,
said method comprising the steps of:
reducing the sectional area of said alloy by coldworking, and
followed by the final step of
heattreating said alloy at a controlled temperature of 400 to 600°C for a controlled time period of 10-150 minutes, without mechanically restraining said alloy to a desired shape, whereby said alloy has, in comparison with Ti₅₀Ni₅₀, pseudoelasticity at about 37°C and an increased yield point of elasticity.

2. The method according to claim 1,
wherein the alloy is reduced to wires of 1.3mm in diameter by means of hot working and cold working and thereafter solution treated at 950°C for 10 minutes before the step of reducing the sectional area.

3. The method according to claim 1 or 2,
wherein the step of reducing the sectional area reduces the alloy to wires of 1.0mm,
the step of heattreating said alloy takes place of 500°C for 30 minutes.

4. The method according to one of claims 1 to 3,
wherein the total amount of Ni and C is 50 - 52 atomic percent.

## Patentansprüche

1. Verfahren des Herstellens einer pseudoelastischen Federlegierung, die durch die chemische Formel
Ti_{a-c/2} Ni_{b-c/2} C_{c}
dargestellt wird, bei der a+b=100, b=50-52 und c=0,20-5,0 in Atomprozent ist, wobei das Verfahren die Schritte aufweist:
Verringern der Querschnittsfläche der Legierung durch Kaltverformen, gefolgt von dem letzten Schritt
Wärmebehandeln der Legierung bei einer gesteuerten Temperatur von 400-600°C während einer gesteuerten Zeitdauer von 10-150 Minuten ohne mechanisches Zurückhalten der Legierung in einer gewünschten Form, wodurch die Legierung im Vergleich mit Ti₅₀ Ni₅₀ Pseudoelastizität bei ungefähr 37°C und einen erhöhten Fließpunkt der Elastizität erhält.

2. Verfahren nach Anspruch 1,
bei dem die Legierung auf Drähte von 1,3mm im Durchmesser mittels Warmverformung und Kaltverformung reduziert wird und danach lösungsbehandelt bei 950°C während 10 Minuten behandelt wird, bevor der Schritt der Verringerung der Querschnittsfläche ausgeführt wird.

3. Verfahren nach Anspruch 1 oder 2,
bei dem der Schritt des Verringerns der Querschnittsfläche die Legierung zu Drähten von 1,0mm verringert,
der Schritt der Wärmebehandlung der Legierung bei 500°C während 30 Minuten stattfindet.

4. Verfahren nach einem der Ansprüche 1 bis 3,
bei dem der Gesamtbetrag von Ni und C 50-52 Atomprozent beträgt.

## Revendications

1. Procédé de fabrication d'un alliage de ressort pseudo-élastique représenté par la formule chimique de Ti_{a-c/2}Ni_{b-c/2}C_{c} dans laquelle :
a + b = 100
b = 50-52 et
c = 0,20 - 5,0
en pourcentage atomique,
ce procédé comprenant les étapes de : réduction de la surface de section de l'alliage par traitement à froid et suivi par l'étape finale de traitement à chaud de l'alliage à une température contrôlée de 400 à 600°C pendant une période de temps contrôlée de 10 à 150 minutes, sans contrainte mécanique de l'alliage à une forme désirée, par laquelle l'alliage a - par comparaison avec Ti₅₀Ni₅₀, une pseudo-élasticité à environ 37°C et une limite de résistance d'élasticité augmentée.

2. Procédé selon la revendication 1,
caractérisé en ce que
l'alliage est réduit en fils de 1,3 mm de diamètre à l'aide de traitement à chaud et de traitement à froid et après quoi le procédé le traite à 950°C pendant 10 minutes avant l'étape de réduction de la surface de section.

3. Procédé selon la revendication 1 ou la revendication 2,
caractérisé en ce que
l'étape de réduction de la surface de section entraîne la réduction de l'alliage en fil de 1,0 mm, et
l'étape de chauffage de l'alliage a lieu à 500°C pendant 30 minutes.

4. Procédé selon l'une des revendications 1 à 3,
caractérisé en ce que
la quantité totale de Ni et de C est de 50-52 % atomique.
